# EUROPEAN PATENT SPECIFICATION

(11) **EP 3 260 214 B1**
(45) Date of publication and mention of the grant of the patent: **18.12.2024**
(21) Application number: 16752596.3
(22) Date of filing: 19.02.2016
(51) Int. Cl.: B21D 22/20

(54) **METHOD OF PRESS FORMING METAL SHEET**
VERFAHREN ZUM PRESSFORMEN EINES BLECHS
PROCÉDÉ DE MISE EN FORME À LA PRESSE D'UNE TÔLE

(30) Priority: 19.02.2015 JP 2015031029
(43) Date of publication of application: 27.12.2017
(73) Proprietor: Nippon Steel Corporation, Tokyo (JP)
(72) Inventor: SAITO, Masahiro, Tokyo 100-8071 (JP); YOSHIDA, Tohru, Tokyo 100-8071 (JP)
(74) Representative: Vossius & Partner Patentanwälte Rechtsanwälte mbB
(86) International application number: PCT/JP2016/054936
(87) International publication number: WO 2016/133210

(56) References cited:
- WO-A1-2012/036262
- DE-C1- 10 135 647
- FR-A1- 2 921 889
- JP-A- 2000 197 969
- JP-A- 2007 276 295
- US-A1- 2002 041 050

## Description

### Technical Field

The present invention relates to a method of forming a metal sheet in which no breakage occurs during forming such as by drawing, stretch flanging, bending, and stretch forming and a formed part formed by that method of forming.

### Background Art

Usually, the formability of a metal sheet falls the more the strength of the metal sheet rises. For this reason, when forming a particularly high strength metal sheet, if the portion to be formed cannot plastically deform enough, the internal stress will exceed the breaking yield strength and the sheet will break.

FIG. 1 shows a mode of breakage at a shoulder part of a punch when drawing a metal sheet. The blank material 1 of the metal sheet is drawn by pressing a flange part 1' of a blank material 1 in a die 2 by a blank holder 4 while pressing it by a punch 3. Drawing proceeds by a balance of a breaking yield strength of the blank material 1 at the shoulder part 3' of the punch 3 and the pulling force acting on the flange part 1' of the blank material 1.

Further, when a deformation resistance 6 of the flange part 1' becomes equal to the breaking yield strength of the blank material 1 contacting the shoulder part 3' of the punch 3, the flange part 1' stops deforming (being pulled into the die 2). On the other hand, deformation proceeds at only the portion of the blank material 1 contacting the shoulder part 3' of the punch 3 resulting in breakage.

To avoid breakage when drawing a blank material, a high breaking yield strength of the portion contacting the shoulder part of the punch is important. Up until now, several arts have been proposed for preventing breakage of a blank material at the time of a drawing operation.

PLT 1 proposes a method of press-forming a blank material during which a location of the blank material where a reduction in thickness is anticipated is provided with two or more weld beads and then the press-forming operation is performed.

PLT 2 proposes a tailored blank material for press-forming use excellent in deep drawability obtained by welding a high strength steel sheet having a 15% or more lower strength and sheet thickness than the material at a center part or a 5% or more better ductility than the material of the center part with another steel sheet forming the center part over the entire circumference of a drawn flange part at a part imparting a wrinkle suppressing force at the time of forming at the outside the part becoming the final product after deep drawing.

However, in each of the above arts, at the weld input heat part of the blank material, the material becomes brittle and the material of the blank material becomes uneven, so it is difficult to completely avoid breakage of the blank material at the time of a press-forming operation.

PLT 3 describes a formed member having at least one ridge portion connecting one surface and another surface, wherein the formed member has a reinforcing member which is joined to at least the ridge portion of the formed member by a weld provided on the ridge portion.

### Citation List

### Patent Literature

PLT 1. Japanese Patent Publication No. 10-175024A
PLT 2. Japanese Patent No. 4532709B
PLT 3. WO 2012/036262 A1

### Summary of Invention

### Technical Problem

In general, as techniques for preventing breakage when forming a metal sheet, roughly classified, improvement of the forming process and improvement of the material of the metal sheet may be considered. For example, for improvement of the drawing process, the method of division of the dies and increase of the number of pressing processes may be considered, but with these methods, a rise in the forming costs and fall in the productivity are unavoidable.

PLTs 1 and 2 disclose improvement of the material of the high strength steel sheet by changing (strengthening) the material by partial hardening or bonding with different materials. However, with these methods as well, similarly, a rise in the forming costs and fall in the productivity are unavoidable.

Therefore, the present invention has as its problem preventing a metal sheet from breaking when forming a metal sheet without changing the material of the metal sheet and the forming process and has as its object the provision of a method of forming solving that problem and a formed part formed by that method of forming.

### Solution to Problem

The inventors studied in-depth means for solving the above problem. As a result, the inventors discovered that when forming a metal sheet, if bonding a reinforcement to a portion where breaking yield strength is required, the breaking yield strength at the above portion is improved and breakage can be prevented.

The present invention was made based on the above discovery and is defined in the claims.

### Advantageous Effects of Invention

According to the present invention, when forming a metal sheet, it is possible to raise the breaking yield strength of a portion where breaking yield strength is required, improve the formability of the metal sheet, and prevent breakage during drawing without changing the material of the metal sheet and the forming process.

### Brief Description of Drawings

FIG. 1 is a view showing a mode of breakage at a shoulder part of a punch when drawing high strength steel sheet.
FIG. 2 is a view showing a mode of preventing breakage by bonding a sheet of fiber reinforced plastic with a portion where breaking yield strength is required when drawing high strength steel sheet.
FIGS. 3A and 3B are views showing a mode of bonding a reinforcement comprised of fiber reinforced plastic with a portion where breaking yield strength is required when drawing a high strength steel sheet. FIG. 3A shows the mode of bonding ring-shaped fiber reinforced plastic to a ring-shaped portion where breaking yield strength is required, while FIG. 3B shows a cross-section of a formed part obtained by drawing the blank material shown in FIG. 3A.
FIGS. 4A and 4B are views showing another mode of bonding a reinforcement comprised of fiber reinforced plastic with a portion where breaking yield strength is required when drawing a high strength steel sheet. FIG. 4A shows the mode of bonding ring-shaped fiber reinforced plastic to two ring-shaped portions where breaking yield strength is required, while FIG. 4B shows a cross-section of a formed part obtained by drawing the blank material shown in FIG. 4A.
FIG. 5 is a view showing a mode of bonding reinforcements comprised of divided patches of ring-shaped fiber reinforced plastic at a ring-shaped portion where breaking yield strength is required.
FIG. 6 is a view showing the position of a punch shoulder expected to become a portion where breakage in deep drawing is a concern.
FIG. 7 is a view showing the position of a flange end expected to become a portion where breakage in stretch flanging is a concern.
FIG. 8 is a view showing a position of bending expected to become a portion where breakage in bending is a concern.
FIG. 9 is a view showing a position of a punch stretching portion expected to become a portion where breakage in stretch forming is a concern.
FIG. 10 is a chart showing the flow for determining the position where the reinforcement is bonded when forming a metal sheet of a complicated shape where it is difficult to predict a portion where breaking yield strength will be required.
FIG. 11 is a view showing a method of bonding a sheet of fiber reinforced plastic with a portion of high strength steel sheet where breaking yield strength is required. FIGS. 12A and 12B are views showing the case of a drawing operation without a sheet of fiber reinforced plastic bonded to a portion where breaking yield strength is required when drawing high strength steel sheet and the case of a drawing operation with a sheet of fiber reinforced plastic bonded. FIG. 12A shows the case of a drawing operation without bonding a sheet of fiber reinforced plastic with a portion where breaking yield strength is required, while FIG. 12B shows the case of a drawing operation while bonding a sheet of fiber reinforced plastic with a portion where breaking yield strength is required.

### Description of Embodiments

The method of forming a metal sheet of the present invention is a method of forming a metal sheet comprising drawing a sheet with a reinforcement bonded in advance to a portion where breaking yield strength is required (below, referred to as "a portion where breakage is a concern").

The formed part of the present invention is characterized by being formed by the method of forming of the present invention.

The method of forming of the present invention will be explained based on the drawings.

FIG. 2 shows as one example of the present invention a mode of drawing a high strength steel sheet wherein a sheet of fiber reinforced plastic is bonded with a portion where breaking yield strength is required so as to prevent breakage.

A blank material 1 of a high strength steel sheet is drawn by pressing a flange part 1' of the blank material 1 in a die 2 by a blank holder 4 while pressing it by a punch 3. Drawing proceeds by a balance of the breaking yield strength of the blank material 1 at the shoulder part 3' of the punch 3 and the pulling force acting on the flange part 1' of the blank material 1.

Further, as explained above, when a deformation resistance 6 of the flange part 1' becomes equal to the breaking yield strength of the blank material 1 contacting the shoulder part 3' of the punch 3, the flange part 1' stops deforming (being pulled into the die 2). On the other hand, deformation proceeds at only the portion of the blank material 1 contacting the shoulder part 3' of the punch 3 resulting in breakage (see FIG. 1) .

On the other hand, when drawing high strength steel sheet shown in FIG. 2, a reinforcement comprised of a sheet of fiber reinforced plastic 8 is bonded in advance with a portion 7 where breaking yield strength is required and then the drawing operation is performed.

In drawing the blank material 1, if bonding a sheet of fiber reinforced plastic 8 with a portion where breakage during drawing is a concern, that is, the portion 7 where breaking yield strength is required, the breaking yield strength is improved at the portion 7 where breaking yield strength is required and the blank material 1 will not break during drawing.

FIG. 2 shows a mode of bonding a fiber reinforced plastic sheet 8 so as to surround a bottom part of a drawn part so that during drawing of high strength steel sheet, the fiber reinforced plastic sheet 8 reliably bonds with the portion 7 where breaking yield strength is required and can sufficiently exert the function of improving the breaking yield strength. The mode of bonding the reinforcement to the portion where breaking yield strength is required is not limited to the mode of bonding shown in FIG. 2. Various modes of bonding can be employed so long as reliably bonding the reinforcement with the portion where breaking yield strength is required. This point will be explained later while showing another bonding mode.

The technique of bonding with a formed part a sheet or patch of carbon fiber reinforced plastic (CFRP) formed separately matching the shape of the formed part to improve the mechanical properties or functionality of the formed part or reinforce it has been known (for example, see FY2010 Report on Project for Assisting Advancement of Strategic Basic Technologies, "Research Relating to Press-Forming Technology for CFRP-Metal Hybrid Parts for Automobile Structural Members", and FY2014 Proceedings of the Japanese Spring Conference for the Technology of Plasticity, "Basic Studies on Reinforcing Effect of CFRP Sheet in Impact Bending Deformation in Tubular State").

However, the method of forming of the present invention has as its basic idea bonding a reinforcement with a forming material (blank material) before a forming operation so as to raise the formability of the portion with the sheet or patch bonded to it. On this point, the method of forming of the present invention basically differs from the above technique of bonding a sheet or patch of fiber reinforced plastic to a formed part after the forming operation so as to improve the mechanical properties or functionality of the formed part or reinforce it.

That fact that when forming a blank material 1, if bonding a fiber reinforced plastic sheet with a portion where breakage during forming is a concern, that is, a portion where breaking yield strength is required, the breaking yield strength is improved in a portion where breaking yield strength is required and the blank material will not break during forming is a new discovery obtained by the inventors and is the characterizing feature of the method of forming of the present invention.

FIGS. 3A and 3B show a mode in drawing high strength steel sheet where a patch of fiber reinforced plastic is bonded with a portion where breaking yield strength is required. FIG. 3A shows a mode where a patch of ring-shaped fiber reinforced plastic is bonded to a ring-shaped portion where breaking yield strength is required, while FIG. 3B shows a cross-section of a formed part obtained by drawing the blank material shown in FIG. 3A.

In the blank material 1 shown in FIG. 3A, a reinforcement comprised of a ring-shaped fiber reinforced plastic sheet 8a is bonded so as to cover a portion where breakage during drawing is a concern, that is, a ring-shaped portion abutting against a shoulder part of the punch and requiring breaking yield strength.

As shown in FIG. 3A, when drawing high strength steel sheet, if it were possible to identify before drawing the portion where breakage during drawing is a concern, that is, the portion abutting against the shoulder part of the punch and where breaking yield strength is thus required, it would be possible to bond a sheet of fiber reinforced plastic wider than the width of the identified portion so as to completely cover the identified portion and thereby raise the breaking yield strength and improve the formability at that portion.

As shown in FIG. 3B, in the formed part 1a obtained by drawing the blank material shown in FIG. 3A, no breakage occurs at the portion with which the fiber reinforced plastic sheet 8a is bonded and where breakage during drawing is a concern, that is, the portion abutting against the shoulder part of the punch and where breaking yield strength is thus required.

FIGS. 4A and 4B show another mode when drawing high strength steel sheet where patches of fiber reinforced plastic are bonded to portions where breaking yield strength is required. FIG. 4A shows a mode where patches of ring-shaped fiber reinforced plastic are bonded to two ring-shaped portions where breaking yield strength is required, while FIG. 4B shows a cross-section of a formed part obtained by drawing the blank material shown in FIG. 4A.

In the blank material 1 shown in FIG. 4A, ring-shaped fiber reinforced plastic sheet 8b and 8c are bonded so as to cover the portions where breakage during drawing is a concern, that is, the two ring-shaped portions abutting against the shoulder parts of a punch and requiring breaking yield strength.

As shown in FIG. 4A, when drawing high strength steel sheet, even if there were a plurality of portions where breakage during drawing was a concern, that is, the portions abutting against the shoulder parts of the punch and where breaking yield strength is thus required, if it were possible to identify the positions of those portions, it would be possible to bond a sheet of fiber reinforced plastic so as to completely cover the identified portions and thereby raise the breaking yield strength and improve the formability at those identified plurality of portions.

As shown in FIG. 4B, in the formed part 1b obtained by drawing the blank material shown in FIG. 4A, no breakage occurs at the portions to which the fiber reinforced plastic sheets 8b and 8c are bonded and where breakage during drawing is a concern, that is, two ring-shaped portions abutting against the shoulder parts of the punch and where breaking yield strength is thus required.

FIGS. 3A and 3B and FIGS. 4A and 4B show the case of drawing a circular blank material axially symmetrically, but the blank material is not limited to a circular blank material. Further, the drawing operation is not limited to drawing axially symmetrically.

According to the method of forming of the present invention, the breaking yield strength of a portion where breaking yield strength is required (a portion where breakage is a concern) is improved, so the freedom of shape of the blank material, freedom of the forming mode, and freedom of shape of the formed part are greatly expanded.

In the method of forming of the present invention, when drawing a blank material, if it were possible to identify a portion where breakage is a concern, that is, a portion abutting against a shoulder part of a punch and where breaking yield strength is required, it would be possible to bond a reinforcement so as to cover the identified portion and raise the breaking yield strength and prevent breakage at the above identified portion.

FIGS. 3A and 3B and FIGS. 4A and 4B show the states when bonding reinforcements comprised of ring-shaped sheets of fiber reinforced plastic to portions where breaking yield strength is required. The shape of the reinforcement is not limited to a specific shape and may be suitably set in accordance with the shape, position, etc. of the identified portion where breaking yield strength is required.

FIGS. 3A and 3B and FIGS. 4A and 4B show modes of bonding ring-shaped sheets of fiber reinforced plastic to the outsides of portions where breaking yield strength is required, but the locations of bonding the reinforcement are not limited to the outsides of the portions where breaking yield strength is required. They may be any of the inside, outside, and two sides of the portion where breaking yield strength is required. The locations of bonding the reinforcement may be suitably set according to the shapes, positions, etc. of the portions where breaking yield strength is required.

Furthermore, when bonding a reinforcement to a portion where breaking yield strength is required, it may also be bonded divided into suitable sections.

FIG. 5 shows a mode of bonding a reinforcement comprised of divided sections of ring-shaped fiber reinforced plastic to a ring-shaped portion where breaking yield strength is required. In FIG. 5, the ring-shaped fiber reinforced plastic is divided into four sections. The sections of fiber reinforced plastic 8a' are bonded arranged in a ring shape.

When joining a divided reinforcement, the mode of division may be suitably determined according to the shape, position, etc. of the portion where the specified breaking yield strength is required.

Above, the method of forming of the present invention was explained with reference to the example of a drawing operation. The method of forming of the present invention is not however limited to a drawing operation. It may also be applied to various forming operations such as shown in FIGS. 6 to 9. FIGS. 6 to 9 show portions where breakage is a concern in various forming operations. FIG. 6 shows deep drawing, FIG. 7 shows stretch flanging, FIG. 8 shows bending, and FIG. 9 shows stretch forming. If such general forming operations, a portion where breakage is a concern can be predicted relatively easily.

Specifically, when deep drawing, the portion where breakage is a concern is the punch shoulder 61, with stretch flanging, it is the flange end 71, with bending, it is the bent portion 81, and with stretch forming, it is the punch stretching portions 91. Therefore, before forming the metal sheet, it is sufficient to bond a reinforcement and then performing forming so as to cover a position forming that portion at the time of forming.

When forming a metal sheet of a complicated shape where a portion where breaking yield strength is required would be difficult to predict, as shown in FIG. 10, CAE (computer aided engineering) may be used to predict a portion where thickness would be reduced if not using a reinforcement and where breakage is thus a concern and then forming in the case of bonding a reinforcement at that portion where breakage is a concern may be again analyzed by CAE so as to determine the position for bonding the reinforcement.

The reinforcement is not particularly limited in grade so long as one able to bear the stress applied to the portion where breakage during forming is a concern. If considering the strength and ease of handling, a sheet of fiber reinforced plastic or high strength steel foil is preferably used. The fiber reinforced plastic need only be a plastic reinforced by a fiber. It is not limited to any specific fiber or plastic. As a suitable example, carbon fiber reinforced plastic may be mentioned. As high strength steel foil, steel foil having a tensile strength at ordinary temperature of 600 MPa or more can be illustrated.

When using a reinforcement comprised of fiber reinforced plastic, the fiber reinforced plastic is preferably bonded so that the direction of the fibers runs along the direction in which breaking yield strength is required, specifically, cuts across any crack formed.

The reinforcement is designed to improve the breaking yield strength at the portion where breaking yield strength is required, so a required thickness is necessary, but the material is not limited to a specific thickness. The thickness of the reinforcement may be suitably set considering the grade of the blank material, the mode of drawing, the shape of the formed part, etc.

The formed part obtained by forming a blank material with a reinforcement bonded to the portion where breaking yield strength is required may, depending on the application, be used after removing the reinforcement or may be used with the reinforcement remaining bonded as it is.

For this reason, the bonding strength when bonding a reinforcement with a portion where breaking yield strength is required may be suitably selected in accordance with the application of the formed part.

The method of bonding the reinforcement with a portion where breaking yield strength is required is not particularly limited. When the reinforcement is fiber reinforced plastic, an adhesive or resin is preferably used. The types of the adhesive and resin are not particularly limited. It is also possible to consider whether to remove the reinforcement from the formed part or leave it as it is so as to suitably select the adhesive. If the reinforcement is high strength steel foil and the reinforcement does not have to be removed from the formed part, it may be bonded by diffusion bonding.

Here, the mechanism by which bonding of a reinforcement improves the breaking yield strength and improves the formability will be explained.

In general, when drawing a blank material by a die and a punch, the breaking yield strength Pbreak of the blank material abutting against a shoulder part of the punch can be calculated by the following formula (1) (see Plastic Forming Technology Series 13 "Press Drawing - Process Design and Die Design -" (Corona), page 23): $Pbreak = 2 π {Rt}_{0} F {\left\{2 \left(r+1\right) \left(r+2\right)/3 \left(2r+1\right)\right\}}^{\left(n+1\right) / 2} {\left(n/e\right)}^{n}$ where,
R: radius of punch
t₀: thickness of blank material
r: Lankford value
e: Napier's constant (base of natural logarithm)
F, n: parameters of Swift formula

The breaking yield strength P'break of the blank material when reinforcing by a reinforcement a portion of the blank material where breakage is a concern (portion where breakage during drawing is a concern), that is, a portion abutting against a shoulder part of the punch and where breaking yield strength is thus required, can be calculated by the following formula (2) $P ′ break = Pbreak + 2 π {Rt}_{frp} {TS}_{frp}$
P'break: breaking yield strength of blank material abutting against shoulder part of punch
R: radius of punch
t_{frp}: thickness of reinforcement
TS_{frp}: tensile strength of reinforcement

As shown in the above formula (2), if bonding a sheet or patch of fiber reinforced plastic as a reinforcement with a portion of the blank material where breakage is a concern, the breaking yield strength P'break after bonding will exceed the breaking yield strength Pbreak of the blank material, so it is possible to estimate the improvement in formability at the above portion where breakage is a concern. In this way, the method of forming of the present invention can be theoretically verified.

The method of forming of the present invention exhibits its effect without regard to the worked material, that is, the metal sheet, and the content of the forming operation. In particular, it exhibits a large effect in forming high strength steel sheet with a tensile strength of 590 MPa or more - which tends to become low in formability.

### Examples

Next, an example of the present invention will be explained, but the conditions in the example are an illustration of the conditions employed for confirming the workability and effect of the present invention. The present invention is not limited to this illustration of conditions. The present invention can employ various conditions so long as not deviating from the scope of the present invention as defined by the claims.

### Example

As shown in FIG. 11, on a thickness 1.0 mm, diameter 108 mm blank material (dual phase steel) 112, a thickness 0.7 mm, diameter 58 mm adhesive sheet (polypropylene resin sheet) 113 and thickness 0.23 mm, diameter 58 mm sheet of carbon fiber reinforced plastic 111 were stacked in that order. The assembly was heated by a hot crimping machine 114 at 180°C for 1 minute, then pressed at 0.049 MPa (≅5 tonf/m²) for 1 minute and air-cooled to bond the carbon fiber reinforced plastic 111 with the blank material 112.

The blank material 112 with the carbon fiber reinforced plastic 111 bonded to it was drawn using the punch and die used in the comparative example.

### Comparative Example

A thickness 1.0 mm, diameter 108 mm blank material (dual phase steel) was drawn using the following punch and die:
Punch shoulder: R5
Punch diameter: 50 mm
Die shoulder: R5
Die diameter: 60 mm
Blank holder pressure: 0.098 MPa (≅10 tonf/m²)

The results are shown in FIG. 12. (a) shows the results of a comparative example of drawing a portion where breaking yield strength is required to which a sheet of fiber reinforced plastic is not bonded, while (b) shows the results of an example of drawing a portion where breaking yield strength is required to which a sheet of fiber reinforced plastic is bonded.

### Industrial Applicability

According to the present invention, when forming a metal sheet, it is possible to raise the breaking yield strength of a portion where breaking yield strength is required, improve the formability of the metal sheet, and prevent breakage during forming without changing the material of the metal sheet and the forming process. The present invention exhibits its effect regardless of the worked material, that is, the metal sheet, and the content of the forming operation. In particular, it exhibits a great effect for operations on high strength steel sheet where the formability tends to become low like drawing, stretch forming, stretch flanging, and bending. The present invention has high applicability in industries manufacturing metal products.

### Reference Signs List

- 1.: blank material
- 1'.: flange part
- 1a, 1b.: formed part
- 2.: die
- 3.: punch
- 3'.: shoulder part
- 4.: blank holder
- 5.: breakage
- 6.: deformation resistance
- 7.: portion where breaking yield strength is required
- 8.: sheet of fiber reinforced plastic
- 8a, 8a'.: reinforcement of fiber reinforced plastic
- 8b, 8c.: reinforcement of fiber reinforced plastic
- 61.: punch shoulder
- 71.: flange end
- 81.: bent portion
- 91.: punch stretching portion
- 111.: sheet of carbon fiber reinforced plastic
- 112.: blank material
- 113.: adhesive sheet
- 114.: hot crimping machine

## Claims

1. A method of press forming a metal sheet comprising the steps of bonding a reinforcement (8) to a part of the metal sheet (1) where breakage during forming is a concern and then press forming the metal sheet,
**characterized in that**
when only the metal sheet (1) is formed in the press forming, the part of the metal sheet (1) where breakage during forming is a concern is reduced in thickness and breaks in the press forming,
the reinforcement (8) is a fiber reinforced plastic, and the fiber reinforced plastic is bonded so that the direction of the fibers cuts across any crack formed when the part of the metal sheet (1) breaks.

2. The method of press forming a metal sheet according to claim 1, wherein a computer aided engineering is used to predict the part of the metal sheet (1) where thickness would be reduced if not using a reinforcement and where breakage is thus a concern and then forming in the case of bonding the reinforcement at the part of the metal sheet (1) again analyzed by the computer aided engineering so as to determine the position for bonding the reinforcement.

3. The method of press forming a metal sheet according to claim 1 or 2, wherein the metal sheet is a high strength steel sheet having a tensile strength of 590 MPa or more.

## Patentansprüche

1. Verfahren zum Pressformen eines Blechs mit den Schritten des Verbindens einer Verstärkung (8) mit einem Teil des Blechs (1), an dem Bruch während des Formens zu befürchten ist, und des anschließenden Pressformens des Blechs,
**dadurch gekennzeichnet, dass**
bei ausschließlichem Formen des Blechs (1) beim Pressformen der Teil des Blechs (1), an dem Bruch während des Formens zu befürchten ist, dickenreduziert wird und beim Pressformen bricht,
die Verstärkung (8) ein faserverstärkter Kunststoff ist und der faserverstärkte Kunststoff so verbunden wird, dass die Richtung der Fasern einen Riss schneidet, der gebildet wird, wenn der Teil des Blechs (1) bricht.

2. Verfahren zum Pressformen eines Blechs nach Anspruch 1, wobei ein Computer-Aided Engineering zum Einsatz kommt, um den Teil des Blechs (1) vorherzusagen, an dem die Dicke reduziert würde, wenn keine Verstärkung verwendet wird, und an dem Bruch somit zu befürchten ist, und anschließendes Formen im Fall des Verbindens der Verstärkung am Teil des Blechs (1) mit erneuter Analyse durch das Computer-Aided Engineering, um die Position zum Verbinden der Verstärkung zu bestimmen.

3. Verfahren zum Pressformen eines Blechs nach Anspruch 1 oder 2, wobei das Blech ein hochfestes Stahlblech mit einer Zugfestigkeit von mindestens 590 MPa ist.

## Revendications

1. Procédé de mise en forme à la presse d'une tôle comprenant les étapes de liaison d'un renfort (8) à une partie de la tôle (1) où la rupture pendant la mise en forme est un problème puis de mise en forme à la presse de la tôle,
**caractérisé en ce que**
lorsque seule la tôle (1) est mise en forme dans la mise en forme à la presse, la partie de la tôle (1) où la rupture pendant la mise en forme est un problème est réduite en épaisseur et se rompt dans la mise en forme à la presse,
le renfort (8) est un plastique renforcé de fibres, et le plastique renforcé de fibres est lié de sorte que la direction des fibres coupe toute fissure formée lorsque la partie de la tôle (1) se rompt.

2. Procédé de mise en forme à la presse d'une tôle selon la revendication 1, dans lequel une ingénierie assistée par ordinateur est utilisée pour prédire la partie de la tôle (1) où l'épaisseur serait réduite si aucun renfort n'était utilisé et où la rupture est ainsi un problème, puis la mise en forme en cas de liaison du renfort au niveau de la partie de la tôle (1) à nouveau analysée par l'ingénierie assistée par ordinateur de manière à déterminer la position pour la liaison du renfort.

3. Procédé de mise en forme à la presse d'une tôle selon la revendication 1 ou 2, dans lequel la tôle est une tôle d'acier à haute résistance ayant une résistance à la traction de 590 MPa ou plus.
